

June 24, 1924.

1,498,738

J. E. G. LAHOUSSE

METHOD OF AND APPARATUS FOR COATING WIRES AND THE LIKE

Filed Aug. 30. 1921



INVENTOR:  
By Joseph E. G. Lahousse  
W<sup>m</sup> Wallace White  
ATTY.

## UNITED STATES PATENT OFFICE.

JOSEPH EDOUARD GUSTAVE LAHOUSSE, OF TERNAY, ISERE, FRANCE, ASSIGNOR TO  
SOCIETE CHIMIQUE DES USINES DU RHONE, OF PARIS, FRANCE.

## METHOD OF AND APPARATUS FOR COATING WIRES AND THE LIKE.

Application filed August 30, 1921. Serial No. 496,878.

*To all whom it may concern:*

Be it known that I, JOSEPH EDOUARD GUSTAVE LAHOUSSE, of Ternay, Isere, France, a citizen of the Republic of France, 5 have invented certain new and useful Improvements in Methods of and Apparatus for Coating Wires and the like, of which the following is a specification.

This invention relates to a method of, 10 and apparatus for, evenly coating wires or filaments of metal or other material with substances, for the purpose of electrical insulation, of protection against external influences or simply for the purpose of reinforcement or strengthening.

The filament under tension, and, if need be, straightened by known means, is conducted through the coating substance which has been liquefied in a suitable manner, and 20 is thence led through a tube the internal diameter of which exceeds the gauge of the filament. The length and bore of the tube are each chosen according to the thickness of the desired coating and the nature and 25 the viscosity of the liquefied coating substance or of its solution.

When using certain substances it may be advantageous to widen the inlet mouth of the tube to a slightly funnel shape so as to 30 facilitate the carrying off of the viscous liquid.

During its forward progress, the wire carries off with it the liquid intended for the coating and in so doing fills the tube, 35 or at least the first portion thereof; the friction in the tube brings about perfect evenness in the coating, care must naturally be taken that the wire is kept centrally in the tube.

40 The coated wire as it is about to leave the tube no longer completely fills it, the less so the greater the speed with which the wire is drawn through. By varying the speed the same tube can be therefore used for wires of different diameters.

The object of the tube is to gauge off the coating mass freely carried off by the wire, whereas in known apparatus for coating with india-rubber the wire and the mass 50 are forced forward and through a gauging nozzle independently of one another.

The method permits of the use of highly viscous liquids and thus realizes an economy in solvents; with this method rapid drying 55 is attained and a wire can for example

be coated in a single pass with a layer of acetate of cellulose sufficient for insulating purposes. The coating is completely dry at a few metres from the point of exit so that the wire can be rolled up, if the heating and ventilation of the chamber is done with care. The recovering of the solvent is considerably facilitated thereby.

The advantages of the method disclosed are obvious, when compared with known methods according to which a wire is drawn freely through a solution; in this case a diluted, slightly viscous solution only can be used, as otherwise the solvent would be carried off in too large a quantity whereby 60 rapid drying and evenness in the coating will be prevented; it follows that the drawing through these diluted solutions must be repeated 5 or 6 times in order to attain the desired thickness. When the resins 65 which are generally used are replaced by acetate of cellulose, fresh difficulties arise when employing the old process, for if diluted solutions be used, the solution remains hanging on the wire in the form of small 70 drops, while on the other hand, if concentrated solutions be used the excess of liquid which can take place only in an irregular manner. One is obliged to repeat 75 the procedure several times in order to cover up and rectify the defects of the one layer 80 by a fresh coating.

Moreover, if a volatile solvent be used in the old process the outlet mouth of the tube 85 becomes cemented up immediately the movement of the wire ceases, if only for a moment. The carrying off of the coating would therefore be prevented and the wire, upon again entering into movement, would 90 come out naked.

In order to obviate this drawback it is advantageous to fit the outlet mouth of the tube within a small closed chamber out of which the wire passes through a fine opening, the walls of which moreover should not touch the wire; this closed chamber thus remains saturated with vapours from the solvent. A small container filled with solvent 100 can also be arranged in this chamber and thus enable the drawing of a wire to be interrupted during a longer period without obstruction being set up.

Referring to the drawing filed herewith, illustrating one particular arrangement of 110

- the apparatus designed according to this invention:
1. *a* is a loose spool to support the wire to be coated.
2. *b* an apparatus of a known type for straightening the wire.
3. *c* the container for the coating fluid.
4. *d* a tube.
5. *e* is a sleeve made of flexible material which represents the chamber saturated with vapours and which permits the tube connected therewith to be centered by means of an adjusting device.
6. *f* is a pipe in which the coated wire is dried by warm air; this can be effected electrically or otherwise. The air charged with the vapour of the solvent is withdrawn through *g* for the purpose of recovering the latter.
7. *h* is a roller the groove in which corresponds with the diameter of the wire.
8. *i* is a spool upon which the coated wire is rolled.
9. The rotation of this spool by mechanical means results in the drawing of the wire through the whole system.
10. *k* is a plug which closes the vapour saturated chamber with the exception of a fine opening.
11. The apparatus as a whole must be so arranged that the wire can easily be renewed, it must also at all points be easily accessible so as to allow of repairing without difficulty in case of accidental breaking.
12. The bore of the tube must be so chosen that thickened portions of the wire, where it has been repaired or knotted, will also pass through without stoppage.
13. The method is not restricted to the use of volatile solvents. It is applicable to all substances which can in any manner whatsoever be liquefied. For example liquefaction may be effected by heat; hardening then follows by cooling during the outward passage through the pipe. In this case devices for the heating and the cooling must be provided. The liquid employed for coating can also be transformed into a hard mass by means of the action of liquids or gases.
14. When employing a solution, the solvent need not necessarily be removed by evaporation as in the example set forth. It can just as well be removed by causing the coated wire to pass through a suitable liquid.
15. What I claim and desire to secure by Letters Patent is:
1. A process for coating wires, filaments or the like, which consists in passing the wire through a liquefied coating substance while maintaining said wire out of contact with any apparatus parts from the moment it enters the said coating substance until the coating on the wire is dry, and then passing the wire through a gauge tube, the thickness of the coating being regulated by the bore of said gauge tube and the speed of the wire.
  2. An apparatus for coating wires, filaments and the like, comprising a container for a liquefied coating substance, a gauge tube of suitable diameter, a vapor chamber and a drying tube co-axially adjustable with said tube, and means external to the apparatus for guiding the object to be coated centrally through the gauge tube, vapor chamber and drying tube without allowing any contact with any part of the apparatus.
  3. An apparatus for coating wires, filaments and the like, comprising a container for a liquefied coating substance, a gauge tube of suitable diameter the inlet of which is funnel-shaped, a vapor chamber and a drying tube co-axially adjustable with said tube, and means external to the apparatus for guiding the object to be coated centrally through the gauge tube, vapor chamber and drying tube without allowing any contact with any part of the apparatus.
  4. An apparatus for coating wires, filaments and the like, comprising a container for a liquefied coating substance, a gauge tube of suitable diameter, a vapor chamber and a drying tube co-axially adjustable with said tube, a heating coil surrounding said drying tube, and means external to the apparatus for guiding the object to be coated centrally through the gauge tube, vapor chamber and drying tube without allowing any contact with any part of the apparatus.
  5. An apparatus for coating wires, filaments and the like, comprising a container for a liquefied coating substance, a removable gauge tube of suitable diameter, a vapor chamber and a drying tube co-axially adjustable with said tube, and means external to the apparatus for guiding the object to be coated centrally through the gauge tube, vapor chamber and drying tube without allowing any contact with any part of the apparatus.

In testimony whereof I have signed my name to this specification.

JOSEPH EDOUARD GUSTAVE LAHOUSSIE.